

No. 806,046.

PATENTED NOV. 28, 1905.

R. BAGGALEY & C. M. ALLEN.  
METHOD OF CONVERTING MATTE.  
APPLICATION FILED AUG. 15, 1904. RENEWED APR. 6, 1905.

2 SHEETS—SHEET 1.

Fig. 2.



Fig. 1.



WITNESSES

Warren M. Gwartz  
A. F. M. Conlin

INVENTORS

Ralph Baggaley  
C. M. Allen  
by B. A. Kendall, B. Byrnes  
Their Attorneys

No. 806,046.

PATENTED NOV. 28, 1905.

R. BAGGALY & C. M. ALLEN.

METHOD OF CONVERTING MATTE.

APPLICATION FILED AUG. 15, 1904. RENEWED APR. 8, 1905.

2 SHEETS—SHEET 2.

Fig. 4.



Fig. 3.



WITNESSES

Warren W. Schwartz.  
J. F. M. Donon.

INVENTORS

Ralph Baggaley  
C. M. Allen  
by Bacheall & Bynes  
their Attorneys

# UNITED STATES PATENT OFFICE.

RALPH BAGGALEY, OF PITTSBURG, PENNSYLVANIA, AND CHARLES M. ALLEN, OF LOLO, MONTANA; SAID ALLEN ASSIGNOR TO SAID BAGGALEY.

## METHOD OF CONVERTING MATTE.

No. 806,046.

Specification of Letters Patent.

Patented Nov. 28, 1905.

Original application filed July 18, 1904, Serial No. 217,112. Divided and this application filed August 15, 1904. Renewed April 6, 1905. Serial No. 254,118.

*To all whom it may concern:*

Be it known that we, RALPH BAGGALEY, of the city of Pittsburgh, in the county of Allegheny and State of Pennsylvania, and CHARLES M. ALLEN, of Lolo, in the county of Missoula and State of Montana, have invented a new and useful Method of Converting Matte, of which the following is a full, clear, and exact description, reference being had to the accompanying drawings, forming part of this specification, in which—

Figure 1 is a vertical longitudinal section of a converter suitable for practice of our invention. Fig. 2 is a vertical cross-section on the line II II of Fig. 1, and Figs. 3 and 4 are like views showing a modification.

The present specification is a division of an application, No. 217,112, filed by us on July 18, 1904.

20 The object of our invention is to reduce the cost of producing blister-copper by eliminating the present heavy expenses for converter-linings and to transform this serious expense into a source of profit, thus constituting a new method of converting mattes.

In the practice of our invention three things are of importance: first, that the converter-walls should be either composed of heavy metal blocks of such relative thickness that 30 they cannot be destroyed during the process or preferably of heavy metal blocks with a light basic interior lining which will also resist injurious action by the oxidized iron, such as must always result where silica is 35 used in direct contact with matte that contains iron and also to the end that the converter-walls may be comparatively clean and hot after the layer of ore has been consumed and dissolved by the action of the matte and 40 heat; second, that the converter shall be so designed and made of such materials that it may be able to withstand without injury the great heat of the process, as well as the intensely corrosive action of the fiery low- 45 grade matte; third, that the converter may be able to withstand this exacting service without unduly abstracting and dissipating the internal heat that is generated by and that is essential to the success of the process.

50 The apparatus which we prefer to use in practicing our invention is composed of heavy metal blocks whose thickness bears a proper

relative proportion to the molten bath to be held, as fully explained in the application, Serial No. 200,943, filed March 31, 1904.

55

The water-jacketed converter shown in Figs. 3 and 4 can be used in practicing this art; but we recommend that at the later stages of the process the flow of water through the jackets be greatly reduced or preferably 60 shut off altogether for a time in order to prevent any excessive abstraction of heat from the vessel.

Many efforts have been made in the past to utilize mineral-bearing ores as the source of 65 silica for fluxing the iron of copper matte after the latter has been oxidized by the converting-blast. As a rule these efforts have taken the form of the use of pulverized ores mixed with clay or some other bonding agent 70 and water into a plastic mass with which the converter is lined. In John Holway's patent, No. 234,129, dated November 9, 1880, a process is described wherein silicious and slag-producing materials are added to the matte. 75 Metalliferous substances containing the necessary slag-producing materials and containing also valuable metals in such small quantities as to make them unfit for treatment by themselves were described as preferable. In 80 actual work John Holway reported to the London Society of Arts that he used quartz sand impregnated with about five per cent. of 85 oxid of iron. He fed this with a shovel into the converter's mouth, but without success. 85

Attempts have been made to supply silica or silicious ore in pulverized form by injecting it with the blast into the molten bath; but this process has not been successful. It has also been proposed to utilize ores that contained not less than eighty-five per cent. of 90 silica and whose distinctive feature was silver values, and to each ton of pulverized argentiferous quartz to add one hundred and seventy-five pounds of fire-clay with suitable 95 proportions of water to make a plastic lining for the converter to flux the oxidized iron of the molten bath. This process has also remained to the present day unused.

At Aguas Calientes a very unusual ore obtained from the St. Gertrude mine in Pachuca, Mexico, has been utilized as a successful converter-lining and fluxing agent. This ore contains approximately eighty per cent. of

pure quartz, twenty per cent. of almost pure alumina, and from eight dollars to fifteen dollars per ton in gold values, which latter are finely and evenly disseminated through the 5 quartz. The ore is pulverized in Chilean mills, is then mixed with suitable proportions of water, and in this form it is rammed as a lining into very large converter-shells, usually to a thickness of about twenty-four inches. 10 It has also been proposed, though without success, to feed white hot silica into the mouth of the converter.

In the process described in a patent of Ralph Baggaley, No. 746,241, dated December 8, 15 1903, cold silica in solid form was fed into the converter either on top of a clean body of molten converter-matte or preferably into an empty heated converter, where it was agglutinated by auxiliary heat, and thereafter the 20 body of molten converter-matte was poured into the converter upon it. Ralph Baggaley's Patent No. 746,260, dated December 8, 1903, described a like process to that described in No. 746,241, except that it utilized mineral-bearing silicious ores as the fluxing material.

In all former efforts to use ore for converter-linings or to utilize either ore or silica by introducing it through the twyers or into the 30 mouth of the converter the aim has been to satisfy the iron in a high-grade converter-matte, and by this means to increase the percentage of the mineral contents, which would also have the effect of decreasing the volume 35 of the molten bath correspondingly through the separation of slag. All such attempts to use ores for lining have been very costly, because such ores must be first pulverized, which in itself is very expensive, then thoroughly 40 mixed with water and, with one exception, with clay, and thereafter they must be tamped or compacted into the converter-shell with rammers, in order that they would remain firmly in position during the converting process. It has been found that the best results 45 are obtained if only a moderate quantity of water be used; but in order to secure such comparatively dry plastic mixture in its position in the converter-shell a large amount of 50 hand-labor has been required in the work of ramming it. This process has also required the expenditure of money for coke with which to dry out the linings before use, and inasmuch as coke is always expensive in localities 55 where copper ores are treated this has added materially to the cost. In actual practice it is found that only a small proportion of such lining can be used until the destructive action must cease, else the destruction of the metal 60 converter-shell will quickly follow, inasmuch as the corrosive action of the bases is not and cannot be distributed evenly over the surface of the acid lining. On the contrary, the iron of the matte attacks the silica of the lining 65 much more at some places than it does at

others. Hence when it has weakened it at any one point to the extent that the metal shell becomes heated to a red heat further converting action must cease or serious and permanent injury to the shell will result. When a 70 lining thus becomes weakened, it necessitates the removal of a large amount of the same in order to prepare the shell for relining, and the portion removed usually is so permeated with fusible material from the former charges 75 that it is unfit to be used again for a lining material. It must be smelted as a means of recovering its contained values, which process involves additional expense. It is estimated that each converter-lining costs at least forty 80 dollars. If carefully prepared, it may last for from seven to twelve blows; but if carelessly applied it may be destroyed in a single blow or in two or three blows. Under the most favorable circumstances a very large 85 proportion of the material contained in each lining is useless for effective work, because the iron of the matte usually eats holes through certain portions of it, thus rendering the balance useless for fluxing purposes. The life 90 of such a lining will be very largely governed by the care and the uniform ramming exercised by the workmen while placing it in position. The constant aim has been to make the lining as durable as possible as 95 a measure of economy. This has led experimenters to avoid everything that would render the lining friable or easily dissolved by the molten bath, and it has therefore been considered necessary to avoid the use of all 100 ores and all lining materials that carry basic elements or compounds, inasmuch as these would contribute to its rapid destruction. Every other consideration has been sacrificed in the effort to maintain the life of the lining 105 to the utmost. By our invention this practice is entirely reversed. Inasmuch as we depend upon the destruction of the lining material as the means whereby we extract and recover mineral values contained in the 110 ores of which we make the lining economy demands that the destruction be rapid, since in this way a greatly-increased amount of effective work can be accomplished in a given time. Our present invention affords the 115 first method that is adapted to the use of a lining containing ores carrying sulfids of the base metals in combination with silica. 120 For the reasons above stated all past experimenters have been forced to compound 120 their lining material with alumina or some equivalent bonding agent mixed with water, and where ores were used at all as lining material only such were used as contained high percentages of silica and such as contained no metals other than gold or silver, (preferably in a finely-disseminated state.) Ores which contained base metals, sulfids, 125 arsenids, antimonids, or any of the elements or compounds usually found in ores or such 130

as would readily be dissolved, and indeed all ores which contained matte-making elements or compounds, were avoided.

In present practice where mattes are low grade in copper values—say below forty per cent., inasmuch as practically the entire remaining sixty per cent., constituting a much larger proportion of the total bulk of the charge, must be removed in the converting process—it has been found necessary either to add additional matte in the molten state from time to time or else to combine charges of matte by transferring partially-blown charges from one converter into another as a means of securing sufficient material with which to finish a charge to blister copper.

In the Bingham Cañon district in Utah many vast bodies of low-grade sulfid ores are found ordinarily containing mineral values varying from four dollars and fifty cents to five dollars and eighty cents per ton. The proportion of copper amounts to one or 1.5 per cent. and the remaining values consist usually of gold and to a small extent of silver. In a single instance ores of this character contained total values of seventeen dollars per ton, the copper varying from one to two per cent. and the remaining values consisting principally of gold and silver. These ores at present are smelted in the ordinary water-jacketed blast-furnace with coke and with slow smelting as a means of enriching them as much as possible before fusion. The resulting matte after the first fusion in the blast-furnace, containing from eight to ten per cent. of material values, is transferred to a number of silica-lined converters, and it causes a rapid destruction of their linings, owing to the heavy percentage of iron. A large proportion of worthless slag is produced, and the proportion of resultant concentrated matte is consequently extremely small. In order to conduct this tedious process on commercial lines, it has been found necessary to transfer these small amounts of concentrated matte from a number of different converters into one in order to produce one full molten bath of, say, forty to fifty per cent. converter-matte, and after consolidating many such charges they are thereafter brought up to the grade of blister-copper in a single silica-lined converter.

By our present invention we depart widely from prior practice, because we utilize as a fluxing agent ores that carry varying percentages of bases, sulfids, and basic compounds. We thus establish the conditions necessary to furnish a constantly-increasing supply of matte of general composition, and we gradually and constantly add percentages of mineral values to our matte, so that we are enabled either to finish the process or, if desired, to bring up the grade of our matte to forty or fifty per cent. of copper, or to even a higher grade, if such is desired. This produces what

is commonly called "converter-matte" without resorting to any of the present wasteful and expensive processes of concentration by water or by fire. In prior processes ores have, with the one exception herein referred to, 70 been unfit for use as lining, for the reason they all contain percentages of basic elements or compounds and are hence unfit for lining converters on the lines of present practice. The reason that an ore lining for converters 75 has been successful at Aguas Calientes, in Mexico, the one exception above referred to, is because the very unusual ore there used is practically free from all basic elements or compounds excepting alumina. In our present invention we can successfully use ores carrying large percentages of bases and basic sulfids, and the presence of these hitherto objectionable elements and compounds will materially contribute to the speed and to the 80 success of the process and will augment the mineral values contained in the bath. We are enabled to add copper, iron, sulfids, gold, silver, and any matte-making elements or compounds by means of our lining, and any 85 and all copper, gold, and silver thus contributed to the bath through the medium of our lining will add to the enrichment of our matte.

In practicing our invention we take a converter, such as shown in Figs. 1 and 2, made 90 of thick metal blocks 2 and lined with a compact inner lining 5, of silica or silica bricks. We apply to the interior surface of this lining a body or coating *c* of copper ores containing silica and containing also sulfids of iron, 100 copper, &c., and preferably gold, silver, and matte-making elements or compounds. We prefer to apply this lining by distributing on the interior of the converter a coating of slag or matte in a liquid condition and then to 105 apply the ore lining to the coated interior and to cause it to adhere thereto, after which it may, if desired, be cemented with another addition of slag or matte. The converter being in a heated condition, we run into it 110 from a smelting-furnace, forehearth, or other convenient source a body of molten slag, preferably enough to equal in volume one-half the usual converter charge, or we may use for this purpose some molten matte. We 115 then tip the converter back and forth on its axis, so as to distribute this slag or matte over the interior surface in a sticky layer *b*, and we then tip the converter completely to discharge the surplus. The body of ore is then 120 added to the converter, and by rocking the latter back and forth it is tumbled over the layer *b* and caused to adhere thereto in a layer *c*, or, if desired, the ore may be spread over the converter with a shovel or otherwise. A 125 small quantity of molten matte or slag is then preferably poured into the converter and, being distributed in like manner over the lining, completes the bonding of the ore particles. The slag or matte quickly sets, and, if desired, 130

this setting can be hastened by blowing air thereon from the twyers 3. The ore is thus held to the converter with sufficient security to serve as a lining and to supply the flux to the charge beneath the bath; but, being open and unpacked, the lining acts more readily and causes the converting operation to proceed more quickly than is possible with linings heretofore employed.

10 Instead of first distributing a layer of molten matte or slag over the converter before applying the lining material we may place such material in the converter and cause it to adhere thereto by pouring upon it a small volume of molten slag or matte.

15 The lining may be constituted by selecting such ores as contain a sufficient quantity of flux, such as oxids or sulfids, to enable the lining to be cintered in place by the application of external heat from oil-burners or the like.

20 Instead of using a converter made of metal blocks, as shown in Figs. 1 and 2, we may employ the converter shown in Figs. 3 and 4, 25 having an exterior water-jacket 4 and an interior compact lining 5, of silica or silica bricks, within which the layer *c* of ore is applied. We show in all these figures burners 7 for supplying flame by which the ore lining may 30 be cintered in place. These burners may be omitted when the ore-body is cemented to the interior walls by molten matte or slag.

35 The quantity of ore employed as lining material is selected with reference to the composition of the matte to be treated. It should contain sufficient silica to flux all the ore contained in the matte that is delivered into the converter, as well as the additions thereto supplied by the fusing of the matte-making 40 compounds introduced with the ore. The amount of ore is preferably so determined that the entire mass will be consumed in a single blow of the converter. It will be patent to those who are conversant with the art 45 of converting that every substance added to

the charge as slag-making material will absorb and will carry away with it an appreciable amount of copper and that the more foreign material that is introduced into the slag the greater will be the loss of copper. 50 It then follows that any additions of silicious or of aluminous substances will aggravate such copper losses in exact proportion to the amount of such additions.

There is no known way, either by fire, by 55 water, or by leaching, commercially speaking, whereby the silica contained in sulfid ores can be removed from the ore without a corresponding loss of the sulfids themselves. Therefore any method that enables the operator to use the same kind of ore for the converter-lining that is used to produce the matte to be converted must effect an important saving in all of the values that would be stolen by substances used for lining that are derived 60 from other sources than the matte-making ore itself.

65 In the converting process as conducted by us in a converter having a compact silica lining within which the body of ore is applied the bath will attack the loose lining of ore so much more rapidly than it can attack the compacted silica that the latter will not be quickly destroyed.

70 We claim—

75 The method herein described of converting matte, which consists in applying to a compact silicious converter-wall, a loose lining containing matte-making compounds and silica in amount sufficient to flux the compounds of 80 the matte to be fluxed, charging matte into the converter and subjecting the same to a blast of air; substantially as described.

70 In testimony whereof we have hereunto set our hands.

RALPH BAGGLEY.  
CHARLES M. ALLEN.

Witnesses:

WILLIAM M. KIRKPATRICK,  
W. D. KYLE.